

# United States Patent

[19]

Shiba et al.

[11] 3,840,373

[45] Oct. 8, 1974

[54] GREEN SENSITIVE SILVER HALIDE  
PHOTOGRAPHIC EMULSION

[75] Inventors: Keisuke Shiba; Masanao Hinata;  
Yasushi Oishi; Yoshinobu Yoshida,  
all of Kanagawa, Japan

[73] Assignee: Fuji Photo Film Co., Ltd.,  
Kanagawa, Japan

[22] Filed: Dec. 1, 1971

[21] Appl. No.: 203,541

[30] Foreign Application Priority Data

Dec. 1, 1970 Japan ..... 45-106113

[52] U.S. Cl. ..... 96/77, 96/99, 96/124

[51] Int. Cl. ..... G03c 1/40, G03c 1/10, G03c 1/14

[58] Field of Search ..... 96/124, 77, 3, 29 D, 99,  
96/137

[56]

## References Cited

### UNITED STATES PATENTS

|           |         |                           |        |
|-----------|---------|---------------------------|--------|
| 2,973,264 | 2/1961  | Nys et al. ....           | 96/124 |
| 2,983,606 | 5/1961  | Rogers ..... 96/29 D      |        |
| 3,173,791 | 3/1965  | Kalenda ..... 96/137      |        |
| 3,397,060 | 8/1968  | Schwan et al. .... 96/124 |        |
| 3,415,646 | 12/1968 | Land ..... 96/29 D        |        |
| 3,663,210 | 5/1972  | Sato et al. .... 96/124   |        |

Primary Examiner—David Klein

Assistant Examiner—Richard L. Shilling

Attorney, Agent, or Firm—Sughrue, Rothwell, Mion,  
Zinn & Macpeak

[57]

## ABSTRACT

A silver halide photographic sensitive material having a green sensitive layer and suitable for use in the diffusion transfer method is disclosed.

8 Claims, 2 Drawing Figures



PATENTED OCT 8 1974

3,840,373

FIG.1



FIG.2



# GREEN SENSITIVE SILVER HALIDE PHOTOGRAPHIC EMULSION

## BACKGROUND OF THE INVENTION

### 1. Field of the Invention

This invention relates to a photographic sensitive material which contains dye developers suitable for the diffusion transfer method and which is spectrosensitized. The invention relates more particularly to a green sensitized sensitive material.

### 2. Description of the Prior Art

Compounds containing a moiety having a dyeing function and a moiety having a development function for silver halide in the same molecule are necessary among photographic elements for forming color images according to the diffusion transfer process. Such compounds are known in general as "dye developers."

It has been reported in U.S. Pat. No. 2,983,606, British Pat. No. 804,971 and French Pat. No. 1,313,767 that when a sensitive element containing a dye developer and silver halide is exposed to light and treated with an alkaline treatment composition, development proceeds in the exposed area, the dye developer is changed so as not to diffuse substantially whereas the developer may diffuse in the unexposed area, and the element is contacted to an image-receiving element to yield a dye transfer image resulting in a positive image in which the density of the image is adversely proportional to the amount of exposure.

The dye developers to be used in this invention are described in the literature. The dye developers may not diffuse substantially in a colloid layer such as a hydrophilic organic colloid which is used at a neutral pH-value in a photographic emulsion but diffuse in such emulsion in the presence of alkaline treatment solution. Available dye developers are described in many patent specifications, for example, Australia Pat. No. 220,279; German Pat. No. 1,036,640; British Pat. Nos. 804,971; 804,973, 804,974 and 804,975; Belgian Pat. No. 554,935; French Pat. Nos. 1,168,292 and 1,313,765; Canadian Pat. Nos. 577,021 and 579,038; and U.S. Pat. Nos. 3,320,063, 3,255,001, 2,992,106, 3,297,441, 3,134,762, 3,236,643, 3,134,763, 3,236,645, 3,134,764, 3,134,672, 3,134,765, 3,183,089, 3,135,734, 3,135,604, 3,173,906, 3,222,169, 3,183,090, 3,201,384, 3,246,985, 3,208,991, 3,142,565, 3,218,312, 3,230,086, 3,262,924, 3,275,617, 3,077,402, 3,282,913, 3,141,772, 3,299,041, 3,309,199, 2,983,605, 3,047,386, 3,076,820, 3,173,929, 3,230,083, 3,236,864, 3,239,339, 3,252,969, 3,253,001, 3,288,778, 3,209,016, 3,135,606, 3,076,808, 3,126,280, 3,236,865, 3,135,605, 3,255,205, 3,131,061, 3,347,673, 3,347,672, 3,246,016, 3,245,790, 3,086,005, 3,295,973, 3,307,947, 3,230,082, 3,230,085, 3,019,107, 3,019,254, 3,022,354, 3,256,269, 3,230,084, 3,232,995, 3,236,873, and 3,252,990.

In general, as mentioned above, the dye developer is a compound which contains the dyeing moiety and at least one silver halide developing group in the same molecule. The term "silver halide developing group" means a group which is suitable for the development of exposed silver halide. The preferred silver halide developing group is the hydroquinonyl group. The developing group may also be o-dihydroxyphenyl or o- and p-

amino-substituted hydroxyphenyl groups. In general, the developing group contains a benzenoid developing group, i.e., aromatic developing group which forms a quinonoid, i.e., a quinone substance in the oxidation.

5 The dyeing moiety of typically available dye developers is the azo or anthraquinone dyeing moiety. In the description of this invention, the dye developers having the azo dyeing moiety are referred to as the azo developers and those having the anthraquinone dyeing moiety as anthraquinone dye developers.

As is well known in the field, dye developers represented by azo or anthraquinone dye developers reduce the sensitivity of silver halide photographic emulsions and especially the spectrosensitized silver halide emulsions (in this case, the absorption due to the dye developer is subtracted). The reduction of sensitivity due to the dye developer is observed not only in the direct addition of the dye developer to the green spectrosensitized silver halide emulsion but in the indirect addition of the dye developer to the green sensitive emulsion layer, i.e., in the contact of the dye developer layer to said sensitive layer. In the latter case, a part of the dye developer in the dye developer layer may diffuse into the sensitive layer.

### 25 3. Objects of the Invention

Accordingly, an object of this invention is to provide a green sensitive layer for a silver halide photographic sensitive material having a high green sensitivity in the presence of a dye developer.

30 More particularly, an object of this invention is to provide a silver halide photographic sensitive material having a green sensitive layer and being suitable for the diffusion transfer method.

Other objects of the invention will be apparent to those skilled in the art as the description of the invention proceeds.

## BRIEF DESCRIPTION OF THE DRAWINGS

FIG. 1 is a sectional view showing an embodiment of a process for obtaining a monochromatic diffusion transfer image.

40 FIG. 2 shows a sectional view of an embodiment of a photographic material to be used for obtaining a multi-color diffusion transfer image.

45 The objects of this invention may be accomplished by including in a silver halide emulsion the combination of at least one of at least two kinds of dyes of three sensitizing dyes represented by the following general formulae (I), (II) and (III):



55 wherein R represents hydrogen atom or lower alkyl ( $\text{C}_{1-3}$ ) such as methyl, ethyl, etc.

60  $\text{Y}_1$  and  $\text{Y}_4$  each represent a hydrogen atom, lower alkyl such as methyl, ethyl, etc., halogen atom such as chlorine and bromine, hydroxyl, alkoxy such as methoxy, ethoxy, etc., amino group such as amino group, methyl amino group, etc., acylamido group such as acetamido group, etc., alcyloxy group such as acetoxyl group, etc., carbalkoxy group such as carbethoxy group, etc., and alkoxy carbonyl amino group such as ethoxycarbonyl amino group.

$Y_2$  and  $Y_5$  each represent a hydrogen atom, lower alkyl such as methyl, ethyl, etc., halogen atom such as chlorine, bromine and fluorine, hydroxyl group, alkoxy such as methoxy, ethoxy, etc., amino group such as amino group, methyl amino group, etc., acylamido group such as acetamido group, etc., acyloxyl group such as acetoxy group, etc., carbalkoxy group such as carbethoxy group, etc., alkoxy carbonyl amino group such as ethoxycarbonyl amino group, etc., and phenyl radical.

$Y_3$  and  $Y_6$  each represent a hydrogen atom or the atomic grouping necessary for the formation of a benzene ring through the connection of  $Y_3$  with  $Y_2$  or of  $Y_6$  with  $Y_5$ .  $Y_2$  and  $Y_5$  each can be connected with  $Y_1$  or  $Y_4$  respectively to form a benzene ring excepting, of course, that both  $Y_3$  with  $Y_2$  and  $Y_2$  with  $Y_1$  form at the same time a benzene ring or both  $Y_6$  with  $Y_5$  and  $Y_5$  with  $Y_4$  form at the same time a benzene ring.

$R_1$  and  $R_2$  each represent an alkyl group such as methyl, ethyl, n-propyl, etc., substituted alkyl radical, which is used in general for cyanine dyes, such as hydroxalkyl (for example, 2-hydroxyethyl, 4-hydroxybutyl, etc.), acetoxyalkyl (for example, 2-acetoxyethyl, 3-acetoxypropyl, etc.), alkoxyalkyl (for example, 2-methoxyethyl, 4-butoxybutyl, etc.), alkyl radical containing carboxyl group (for example, 2-carboxyethyl, 3-carboxypropyl, 2-(2-carboxyethoxy)ethyl, etc.), alkyl radical containing sulfo group (for example, 2-sulfoethyl, 3-sulfopropyl, 3-sulfobutyl, 4-sulfobutyl, 2-hydroxy-1-sulfopropyl, 2-(3-sulfopropoxy)ethyl, 2-acetoxy-1-sulfopropyl, 3-methoxy-2-(3-sulfopropoxy)propyl, 2-(2-(3-sulfopropoxy)ethoxy)ethyl, 2-hydroxy-3-(3'-sulfopropoxy)-propyl, etc.), aralkyl (for example, benzyl, phenylethyl, p-sulfonylbenzyl, p-carboxybenzyl, p-sulfophenethyl or allyl radical), and at least one of  $R_1$  and  $R_2$  is an alkyl radical containing a carboxyl or sulfo group.

$X$  represents an anion such as chloride, bromide, iodide, thiocyanate, sulfonate, perchlorate, p-toluenesulfonate, methylsulfonate, ethylsulfate, etc., and  $n$  represents 1 or 2, wherein  $n = 1$  when said dye forms an intramolecular salt.



wherein  $R_3$  represents a lower alkyl such as methyl, ethyl, etc. or allyl radical.

$Y_7$  represents a hydrogen atom or halogen atom such as chlorine, bromine or fluorine.

$Y_8$  represents a hydrogen atom, a halogen atom such as chlorine, bromine and fluorine, etc., alkoxy group such as methoxy, ethoxy, etc., amino group such as amino, methyl amino, etc., acylamido group such as acetamido, etc., acyloxyl group such as acetoxy, etc., alkoxy carbonyl amino group such as ethoxycarbonyl amino, etc.

$Y_9$  represents a hydrogen atom, lower alkyl radical such as methyl, ethyl, etc., halogen atom such as chlorine and bromine, hydroxyl and alkoxy group such as methoxy, ethoxy, etc.

$Y_{10}$  represents a hydrogen atom, lower alkyl radical such as methyl, ethyl, etc., halogen atom such as chlorine, bromine and fluorine atom, alkoxy group such as

methoxy, ethoxy, etc., phenyl, substituted phenyl such as p-sulfophenyl, etc., carboxyl group, alkoxy carbonyl group such as methoxycarbonyl, ethoxycarbonyl, etc., cyano group and trifluoromethyl group.  $Y_{11}$  represents a hydroxyl group or an atomic grouping which is connected to  $Y_{10}$  to form a benzene ring.  $Y_9$  and  $Y_{10}$  may be connected to form a benzene ring, excepting that both  $Y_9$  with  $Y_{10}$  and  $Y_{10}$  with  $Y_{11}$  form at the same time benzene rings.

10  $R_1$ ,  $R_2$ ,  $X$  and  $n$  have the same meanings as in formula (I).



wherein  $R_4$  and  $R_5$  each represents alkyl radical such as methyl, ethyl, propyl, butyl, etc.;  $Y_{12}$  and  $Y_{14}$  each represents hydrogen atom or halogen atom such as chlorine, bromine, iodine and fluorine;  $Y_{13}$   $Y_{15}$  each represents hydrogen atom, halogen atom such as chlorine, bromine, iodine and fluorine atom, alkoxy group such as methoxy, ethoxy, butoxy, etc., amino group such as amino, methyl amino, dimethyl amino, etc., acylamido group such as acetamido, etc., acyloxyl group such as acetoxy, etc., alkoxy carbonyl amino group such as ethoxycarbonyl amino, etc., cyano group, trifluoromethyl group, alkylsulfonyl group such as methylsulfonyl, etc., sulfamyl group, alkylaminosulfonyl group such as ethylaminosulfonyl, diethylaminosulfonyl, etc., morpholinosulfonyl group and piperidinosulfonyl group; and  $R_1$ ,  $R_2$ ,  $X$  and  $n$  have the same meanings as given in formula (I).

The sensitizing dyes to be used in this invention are known. Dyes represented by the general formula (I) and (III) are the sensitizing dyes described in French Pat. No. 1,108,778 (Sept. 14, 1955), U.S. Pat. No. 2,503,776, U.S. Pat. No. 2,912,329 (Nov. 10, 1959) and U.S. Pat. No. 3,397,060 (Aug. 13, 1968) and can be synthesized readily for those skilled in the art with reference to those patent specifications, and those not described in said patent specifications can also be synthesized readily according to similar methods thereto.

The dyes represented by the general formula (II) are the sensitizing dyes described in the Japanese Publication 14030/69 (Jan. 18, 1966) and can be synthesized readily for those skilled in the art in reference to the publication specification, and those not described in the specification can be synthesized readily according to the similar method thereto. The following material is exemplary of methods of preparation of the dyes represented by the general formula (II).

The sensitizing dyes used in the present invention may be prepared by the condensation methods known to those skilled in the art. That is, the unsymmetric carbocyanine dye used in the present invention may be obtained by condensing an acetanilide intermediate compound with a cyclic quaternary ammonium salt having an active methyl group in a solvent such as nitrobenzene, an alcohol or acetic anhydride in the presence of a suitable organic base such as triethylamine or piperidine. In the case of employing an anilino intermediate compound, the dye may be prepared by acetylating the intermediate compound prior to the condensation and

then subjecting thus formed acetanilide intermediate compound in situ to the subsequent condensation reaction.

Examples of sensitizing dyes to be used in this invention are given as follows but it is not intended that this invention be restricted to only these examples.

I-1



I-2



I-3



I-4



I-5



I-6



I-7



II-1



II-2



II-3





11 14



III-1



III-2



三



According to several techniques in the diffusion transfer method, image-forming components which

have been already described hereinbefore can be used to yield a monochromic or multi-color image.

In one method for the formation of a color transfer image by using color developers, at least two selectively sensitized sensitive layers are placed in contact on a support and treated at the same time and without being separated together with a single common image-receiving layer.

FIG. 1 illustrates one embodiment of a method for the formation of monochromatic transfer image. The sensitive element consists of a support 11, a layer containing a color image-forming component 12 and a silver halide emulsion layer 13. Further, a vessel 16 capable of being ruptured and carrying an alkali treating composition is placed on the sensitive element, which is shown apart from the treating composition. On the other hand, an image-receiving element consists of a support 15 and an image-receiving layer 14. After exposure, the image-receiving element is in contact with the sensitive element and the vessel 16 capable of being ruptured is ruptured by applying a suitable pressure, e.g., by progressing between a pair of opposed and suitably grooved rolls (not shown) to spread the liquid treating composition layer-like between said elements. The treating composition penetrates into the silver halide emulsion and develops the latent image contained in the emulsion. The color image-providing component migrates from the unexposed area to the contacted image-receiving element to form a positive color image resulting from the exposure thereon. After at least a part of the color image-forming element is then transferred, the image-receiving element is removed from the contact with the sensitive element.

The silver halide emulsion layer consists of, for example, a blue sensitive silver halide emulsion layer and a green sensitive silver halide emulsion layer, each of said emulsions containing a magenta dye developer and a cyan dye developer respectively. The dye developer can be incorporated in the silver halide emulsion layer (for example, in the form of particles) or contained in a suitable layer below the silver halide emulsion layer. Each combination of the silver halide emulsion layer and the dye developer layer is separated from the other combinations through a suitable intermediate layer, e.g., a gelatin or polyvinyl alcohol layer.

The natural color sensitive material of this type consists of a support carrying a red sensitive silver halide emulsion layer, a green sensitive silver halide emulsion layer and a blue sensitive silver halide emulsion layer, each of said emulsions containing a cyan dye developer, a magenta dye developer and a yellow dye developer. The manner of containing said dye developers is the same as mentioned above.

In a further method for the formation of a multi-color image, a plurality of sensitive elements suitable for the treatment with more than one treating liquid composition in connection to a suitable number of image-receiving layers and suitable dye developers are contained for example in the sensitive elements. Examples of the film constitution of this type are described in U.S. Pat. No. 2,647,049.

In a still further method for the formation of a multi-color image, sensitive silver halide emulsion layers comprising at least two selectively sensitized sensitive micro-elements which are disposed in the form of a sensitive screen are used. For example, each of the sensitive micro-elements contains a suitable dye developer in the silver halide emulsion layer or in the other emulsion layer. For example, the sensitive silver halide layer consists of a sensitive screen of a blue sensitized emulsion micro-element and a green sensitized emulsion mi-

cro-element, each of said elements being in contact with each other in the screen pattern and containing a magenta and cyan dye developer respectively. Sensitive

5 screens suitable for the color photography of subtractive color processes are placed in contact with each other in a screen pattern and consist of red, green and blue sensitive emulsion micro-elements, which are combined with each dye developer for forming cyan, magenta and yellow images, respectively. The transfer method of this type is described in U.S. Pat. Nos. 2,968,554 and 2,983,606.

10 A dye developer which provides cyan, magenta or yellow to the green sensitive emulsion to be used in this invention is used and further dye developers of other colors such as black dye developers as well as a mixture of dye developers may be used.

15 The dye developer to be used in this invention may be introduced into the sensitive element, e.g., each silver halide emulsion, or into the upper or lower layer thereof. The layer of such dye developer may be obtained by coating a solution containing about 0.5 – 8 percent by weight of a dye developer dispersed in a colloidal binder such as gelatin or dissolved in a synthetic polymer binder such as cellulose hydrogenacetate phthalate.

20 The alkali treating composition to be used in this invention is an aqueous solution of at least one alkaline compound such as diethyl amine, sodium or potassium hydroxide or sodium carbonate. When the alkali treating composition is applied by spreading, preferably as a relatively thin uniform layer, the composition can contain viscosity-increasing compounds which may be film-forming materials of such type that may form a relatively hard and stable film when the composition is spread and dried. Preferred film-forming materials are high molecular weight polymers such as water soluble polymeric ethers which are inert to alkaline solutions, e.g., hydroxyethyl cellulose and sodium carboxymethyl cellulose. It is possible to use other film-forming materials of which viscosity-increasing capacities are not substantially affected by standing for a long time in the solution. An alkali treating composition containing mordant can be used also, which is known for example from Japanese Publication No. 6449/63. Examples of suitable alkali treating compositions are described in the examples of the text of this invention. Occasionally, it is desirable to apply the alkali treating composition to the sensitive element prior to the exposure according to the procedure described in U.S. Pat. No. 3,087,816.

25 The alkali treating composition may contain auxiliary developers, i.e., a development accelerator (s) such as p-methylaminophenol, 2,4-diaminophenol, p-benzylaminophenol, hydroquinone, tolhydroquinone, phenyl hydroquinone, 4-methylphenyl hydroquinone and others. As described in U.S. Pat. No. 3,039,869, a plurality of auxiliary developers such as the combination of 3-pyrazolidone and benzenoid developer can be used. As examples of the combination of auxiliary developers, there are mentioned a couple of 1-phenyl-3-pyrazolidone and p-benzylaminophenol as well as of 1-phenyl-3-pyrazolidone and 2,5-bisethylaminohydroquinone. These auxiliary developers are used in the alkali treating composition or at least a part thereof may be contained previously in the silver halide emulsion layer or a layer containing a dye developer. The oxidation-reduction reaction is repeated in the dye developer-auxiliary developer-exposed silver halide system, in which the auxiliary developer serves a catalytic function.

The azo dye developers to be used in this invention are known and described in, for example, U.S. Pat. No. 3,134,672; there is mentioned therein the following compounds:

- (1) 1-phenyl-3-n-carbobutoxy-4-(p-(2',5'-dihydroxyphenethyl)-phenylazo)-5-pyrazolone;
- (2) 1-phenyl-3-(N-2'-ethylhexylcarbamido)-4-(p-(2',5'-dihydroxyphenethyl)-phenylazo)-5-pyrazoline;
- (3) 1-(p-N,N-diethylsulfonamidophenyl)-3-N-n-butylcarbamido-4-(p-(2',5'-dihydroxyphenethyl)-phenylazo)-5-pyrazolone;
- (4) 1-phenyl-3-N-n-hexylcarbamido-4-(p-(2',5'-dihydroxyphenyl-propyl)-phenylazo)-5-pyrazolone;
- (5) 1-phenyl-3-trifluoromethyl-4-(p-(2',5'-dihydroxyphenylisobutyl)-phenylazo)-5-pyrazolone;
- (6) 1-phenyl-3-N-β-hydroxyethylcarbamido-4-(p-(2',5'-dihydroxyphenethyl)-phenylazo)-5-pyrazolone;
- (7) 1-phenyl-3-N-n-hexylcarbamido-4-(p-(2',5'-dihydroxy-4'-methylphenethyl)-phenylazo)-5-pyrazolone;
- (8) 1-phenyl-3-N-n-hexylcarbamido-4-(p-(2',5'-dihydroxyphenethyl)-phenylazo)-5-pyrazolone;
- (9) 1-phenyl-3-N-n-heptylcarbamido-4-(p-(2',5'-dihydroxyphenethyl)-phenylazo)-5-pyrazolone;
- (10) 1-phenyl-3-N-n-hexylcarbamido-4-(p-(2',5'-dihydroxy-4'-chlorophenethyl)-phenylazo)-5-pyrazolone;
- (11) 1-phenyl-3-trifluoromethyl-4-(p-(2',5'-dihydroxyphenethyl)-phenylazo)-5-pyrazolone;
- (12) 1-phenyl-3-phenyl-4-(p-(2',5'-dihydroxyphenethyl)-phenylazo)-5-pyrazolone;
- (13) 1-phenyl-3-N-cyclohexylcarbamido-4-(p-(2',5'-dihydroxyphenethyl)-phenylazo)-5-pyrazolone;
- (14) 1-phenyl-3-N-n-butylcarbamido-4-(p-(2',5'-dihydroxyphenethyl)-phenylazo)-5-pyrazolone;



- (15) 1-phenyl-3-carbethoxy-4-(p-(2',5'-dihydroxyphenethyl)-phenylazo)-5-pyrazolone;
- (16) 1-phenyl-3-methyl-4-(p-(2',5'-dihydroxyphenethyl)-phenylazo)-5-pyrazolone;
- (17) 1-phenyl-3-amino-4-(p-(2',5'-dihydroxyphenethyl)-phenylazo)-5-pyrazolone;
- (18) 2-(p-(2',5'-dihydroxyphenethyl)-o-methylphenylazo)-4-methoxy-1-naphthol;
- (19) 2-(p-(2',5'-dihydroxyphenethyl)-phenylazo)-4-isobutoxy-1-naphthol;
- (20) 2-(p-(2',5'-dihydroxyphenethyl)-phenylazo)-4-N-methyl-N-phenylsulfonamido-1-naphthol;
- (21) 2-(p-(2',5'-dihydroxyphenethyl)-phenylazo)-4-methylsulfon-1-naphthol;
- (22) 2-(m-(2',5'-dihydroxyphenethyl)-phenylazo)-4-n-propoxy-1-naphthol;
- (23) 2-(p-(2',5'-dihydroxyphenethyl)-phenylazo)-4-ethoxyethoxy-1-naphthol;
- (24) 2-(p-(2',5'-dihydroxyphenethyl)-phenylazo)-4-methylsulfide-1-naphthol;
- (25) 2-(p-(2',5'-dihydroxyphenethyl)-phenylazo)-4-β-chloroethoxy-1-naphthol;

- (26) 2-(p-(2',5'-dihydroxyphenethyl)-α-naphthylazo)-4-methoxy-1-naphthol;
- (27) 2-(p-(2',5'-dihydroxyphenylisobutyl)-phenylazo)-4-methoxy-1-naphthol;
- (28) 2-(p-(2',5'-dihydroxyphenylpropyl)-phenylazo)-4-isopropoxy-1-naphthol;
- (29) 2-(p-(2',5'-dihydroxyphenylpropyl)-phenylazo)-4-n-propoxy-1-naphthol;
- (30) 2-(p-(2',5'-dihydroxy-4'-methylphenethyl)-phenylazo)-4-N,N-diethyl-sulfonamido-1-naphthol;
- (31) 2-(p-(2',5'-dihydroxy-3',4'-dimethylphenethyl)-phenylazo)-4-methoxy-1-naphthol;
- (32) 2-(p-(2',5'-dihydroxyphenethyl)-phenylazo)-4-acetyl-1-naphthol;
- (33) 2-(p-(2',5'-dihydroxy-4'-methylphenethyl)-phenylazo)-4-methoxy-1-naphthol;
- (34) 2-(p-(2',5'-dihydroxy-4'-methylphenethyl)-phenylazo)-4-n-propoxy-1-naphthol;
- (35) 2-(p-(2',5'-dihydroxyphenethyl)-phenylazo)-4-β-hydroxyethoxy-1-naphthol;
- (36) 2-(p-(2',5'-dihydroxy-3',4',6'-trimethylphenethyl)-phenylazo)-4-methoxy-1-naphthol;
- (37) 2-(p-(2',5'-dihydroxy-3'-methylphenethyl)-phenylazo)-4-n-propoxy-1-naphthol;
- (38) 2-(p-(3',4'-dihydroxyphenethyl)-phenylazo)-4-n-propoxy-1-naphthol;
- (39) 2-(p-(2',5'-dihydroxyphenethyl)-o-methoxyphenylazo)-4-N,N-dimethyl-sulfonamido-1-naphthol;
- (40) 2-(p-(2',5'-dihydroxyphenethyl)-phenylazo)-4-hexyloxy-1-naphthol;
- (41) 2-(p-(2',5'-dihydroxyphenethyl)-phenylazo)-4-cyclohexyl-1-naphthol;
- (42) 2-(p-(2',5'-dihydroxyphenethyl)-phenylazo)-4-isopropoxy-1-naphthol;
- (43) 2-(p-(2',5'-dihydroxyphenethyl)-phenylazo)-4-n-propoxy-1-naphthol;
- (44) 2-(p-(2',5'-dihydroxyphenethyl)-phenylazo)-4-ethoxy-1-naphthol;
- (45) 2-(p-(2',5'-dihydroxyphenethyl)-phenylazo)-4-methoxy-1-naphthol;
- (46) 2-(p-(2',5'-dihydroxyphenethyl)-phenylazo)-4-acetamido-1-naphthol;
- (47) 2-(p-(2',5'-dihydroxyphenethyl)-phenylazo)-4-amino-1-naphthol;
- (48) 2-(p-(2',5'-dihydroxyphenethyl)-phenylazo)-4-sulfo-1-naphthol;
- (49) 5-amino-8-(p-(2',5'-dihydroxyphenethyl)-phenylazo)-1-naphthol;
- (50) 5-β-hydroxyethylamino-8-(p-(2',5'-dihydroxyphenethyl)-phenylazo)-1-naphthol;
- (51) 4-[(p-(2',5'-dihydroxyphenethyl)-phenylazo)-5-acetamido-1-naphthol];
- (52) 1-(p-(2',5'-dihydroxyphenethyl)-o-methoxyphenylazo)-8-acetamido-2-naphthol;
- (53) 1-(p-(2',5'-dihydroxyphenethyl)-phenylazo)-2-naphthol;
- (54) 4-(p-(2',5'-dihydroxyphenethyl)-phenylazo)-1-N-ethylamino-naphthalene;
- (55) 4-(p-(2',5'-dihydroxyphenethyl)-phenylazo)-1-naphthylamine;
- (56) 4-(p-(2',5'-dihydroxyphenethyl)-phenylazo)-5-hydroxyaceto-naphthalene;
- (57) 8-amino-5-(p-(2',5'-dihydroxyphenethyl)-phenylazo)-quinoline;
- (58) 2,5-dimethoxy-4-(p-(2',5'-dihydroxyphenethyl)-phenylazo)-aniline;

- (59) 2-formyl-4-(p-(2',5'-dihydroxyphenethyl)-phenylazo)-phenol; and  
 (60) 4-(p-(2',5'-dihydroxyphenethyl)-phenylazo)-3-phenyl-isoxazolone-5.
- The anthraquinone dye developers to be used in this invention are known and described in, for example, U.S. Pat. Nos. 2,983,605, 2,983,606, etc.; there are mentioned the following compounds:
- (61) 1,4-bis-(p-(N-(hydroquinonylcarbamylmethyl)-amino)-phenyl-amino)-anthraquinone;  
 (62) 1,4-bis-hydroquinonylcarbamylmethylaminoanthraquinone;  
 (63) 1,4-bis-( $\alpha$ -methyl- $\beta$ -hydroquinonylethylamino)-anthraquinone;  
 (64) 1,4-bis-( $\alpha$ -methyl- $\beta$ -hydroquinonylethylamino)-5,8-dihydroxyanthraquinone;  
 (65) 1,4-bis-( $\alpha$ -methyl- $\beta$ -hydroquinonylpropylamino)-5,8-dihydroxyanthraquinone;  
 (66) 1,4-bis-( $\alpha$ -methyl- $\beta$ -hydroquinonylpropylamino)-anthraquinone;  
 (67) 1,4-bis-hydroquinonylmethylaminoanthraquinone;  
 (68) 1,4-bis-( $\alpha$ -methyl- $\beta$ -hydroquinonylethylamino)-6,7-dichloroanthraquinone;  
 (69) 1,4-bis-( $\alpha$ -methyl-2',5'-dihydroxybenzylamino)-anthraquinone;  
 (70) 1,4-bis-( $\alpha$ -methyl- $\beta$ -hydroquinonylethylamino)-5,8-bis-benzenesulfo-naminoanthraquinone;  
 (71) 1,4-bis-( $\alpha$ -methyl- $\beta$ -hydroquinonylethylamino)-5-hydroxy-8-amino-anthraquinone;  
 (72) 1,4-bis-( $\beta$ -hydroquinonylethylamino)-anthraquinone;  
 (73) 1,4-bis-( $\beta$ -(3',4'-dihydroxyphenyl)-ethylamino)-5,8-dihydroxyphenyl-ethylamino)-5,8-dihydroxyanthraquinone;  
 (74) 1,4-bis-( $\beta$ -(3',4'-dihydroxyphenyl)-ethylamino)-anthraquinone;  
 (75) 1,4-bis-( $\alpha$ -ethyl- $\beta$ -hydroquinonylethylamino)-anthraquinone;  
 (76) 1,4-bis-(2',5'-dihydroxyanilino)-anthraquinone;  
 (77) 1,4-bis- $\beta$ -(homogentisamido)-ethylaminoanthraquinone;  
 (78) 1,4-bis-homogentisamidoanthraquinone;  
 (79) 1,4-bis-(2',5'-dihydroxyanilino)-anthraquinone;  
 (80) 1,4-bis-( $\beta$ -(2',5'-dihydroxyphenyl)-propylamino)-anthraquinone;  
 (81) 1,4-bis-(1',5'-bis-(2'',5''-dihydroxyphenyl)-3'-pentyl)-aminoanthraquinone;  
 (82) N-monobenzoyl-1,4-bis-( $\beta$ -(3',4'-dihydroxyphenyl)-ethylamino)-anthraquinone;  
 (83) N-monobenzoyl-1,4-bis-( $\beta$ -(2',5'-dihydroxyphenyl)-ethylamino)-anthraquinone;  
 (84) 1,4-diamino-N-( $\beta$ -2',5'-dihydroxyphenyl- $\alpha$ -methylethyl)-2,3-anthraquinonedicarboximide;  
 (85) 1-imino-4-hydroxy-N-(62-2',5'-dihydroxyphenyl- $\alpha$ -methylethyl)-2,3-anthraquinonedicarboximide;  
 (86) 1-hydroxy-4-(1',5'-bis-(2'',5''-dihydroxyphenyl)-3''-pentyl)-amino-anthraquinone;  
 (87) 1-amino-4-anilino-2-hydroquinonylsulfamylan-thraquinone;  
 (88) 1-aminoethylamino-4-hydroquinonylcarbamylmethylaminoethyl-aminoanthraquinone;  
 (89) 1-amino-4-(p-(N-hydroquinonylcarbamylmethylamino)-phenylamino)-2-anthraquinonesulfonic acid sodium salt;  
 (90) 1-( $\alpha$ -hydroxymethylpropylamino)-4-( $\alpha$ -methyl- $\beta$ -hydroquinonylethylamino)-anthraquinone;

- (91) 1-( $\alpha$ -hydroxymethylpropylamino)-4-( $\alpha$ -methyl- $\beta$ -hydroquinonylmethyl-amino)-5,8-dihydroxyanthraquinone;  
 (92) 1-hydroxy-4-(2',5'-dihydroxyanilino)-anthraquinone;  
 (93) 1-hydroxy-4-( $\alpha$ -methylhydroquinonylethylamino)-anthraquinone;  
 (94) 1-( $\alpha$ -methyl- $\beta$ -hydroquinonylethylamino)-4-( $\alpha$ -ethyl- $\beta$ -hydroquinonyl-ethylamino)-anthraquinone;  
 (95) 1-( $\alpha$ -methyl- $\beta$ -hydroquinonylethylamino)-4-( $\alpha$ -ethyl- $\beta$ -hydroquinonyl-ethylamino)-5,8-dihydroxyanthraquinone;  
 (96) 1-( $\alpha$ -hydroxymethylpropylamino)-4-( $\alpha$ -methyl- $\beta$ -hydroquinonylethylamino)-5-hydroxyanthraquinone;  
 (97) 1-( $\alpha$ -hydroxymethylpropylamino)-4-( $\beta$ -(4'-methyl-2',5'-dihydroxyphenyl- $\beta$ -methyl-ethylamino)-anthraquinone;  
 (98) 1-ethylamino-4-( $\beta$ -(3',4'-dihydroxyphenyl)-ethylamino)-anthraquinone;  
 (99) 1-chloro-4-( $\beta$ -hydroquinonylethylamino)-anthraquinone;  
 (100) 1-hydroxy-4-( $\beta$ -(3',4'-dihydroxyphenyl)-ethylamino)-anthraquinone;  
 (101) 1-( $\beta$ -hydroxyethylamino)-4-( $\beta$ -hydroquinonylethylamino)-anthraquinone;  
 (102) 1-( $\beta$ -hydroxyethylamino)-4-( $\alpha$ -methyl- $\beta$ -hydroquinonylethylamino)-5,8-dihydroxyanthraquinone;  
 (103) 1-methylamino-4-( $\beta$ -hydroquinonylethylamino)-anthraquinone;  
 (104) 1- $\beta$ -hydroxyethylamino-4-( $\alpha$ -methyl- $\beta$ -hydroquinonylethylamino)-anthraquinone;  
 (105) 1- $\beta$ -aminoethylamino-4- $\beta$ -(homogentisamido)-ethylaminoanthraquinone;  
 (106) 1,5-bis-hydroquinonylmethylaminoanthraquinone;  
 (107) 1,5-bis-( $\beta$ -3',4'-dihydroxyphenyl)-ethylamino-  
 (108) 1,5-bis-( $\beta$ -hydroquinonylethylamino)-anthraquinone;  
 (109) 1,5-bis-( $\alpha$ -methyl- $\beta$ -hydroquinonylethylamino)-anthraquinone;  
 (110) 1,5-bis-homogentisamido-4,8-dihydroxyanthraquinone;  
 (111) 1,5-bis-homogentisamidoanthraquinone;  
 (112) 1,5-bis-(N-methylhomogentisamido)-5,8-dimethylaminoanthraquinone;  
 (113) 1-chloro-5-( $\beta$ -hydroquinonylethylamino)-anthraquinone;  
 (114) 1-( $\beta$ -(3',4'-dihydroxyphenyl)-ethylamino)-5-nitroanthraquinone;  
 (115) 1,8-bis-( $\beta$ -(3',4'-dihydroxyphenyl)-ethylamino)-anthraquinone;  
 (116) 1,8-bis-( $\beta$ -hydroquinonylethylamino)-anthraquinone;  
 (117) 4,8-bis-(2',5'-dihydroxyanilino)-anthraquinone;  
 (118) 4-(2',5'-dihydroxyanilino)-8-chloroanthraquinone;  
 (119) 1-(p-( $\beta$ -hydroquinonylethyl)-phenylamino)-anthraquinone;  
 (120) 1-( $\beta$ -(3',4'-dihydroxyphenyl)-ethylamino)-anthraquinone; and  
 (121) 1-homogentisamido-5-amino-4,8-dihydroxyanthraquinone.

It is known that the sensitizing dyes to be used in this invention are available for the spectrosensitization of conventional silver halide emulsions. Sensitizing dyes which are useful in the use of anthraquinone dye devel-

opers are described in Japanese Pat. Publication 392/65 and contain carboxyalkyl or sulfoalkyl group (the alkylene chain used is n-alkylene). In particular, for the use of anthraquinone dye developers, a sufficient sensitization cannot be obtained without a large amount of sensitizing dye per unit of silver halide because the dye developer is apt to desorb the sensitizing dye from the silver halide. However, when a multi-layer material is prepared with a large amount of sensitizing dye, the sensitizing dye in the green sensitive emulsion layer diffuses disadvantageously into other silver halide sensitive layers (e.g., blue or red sensitive layers), which is accordingly spectrosensitized. In particular, a sensitizing dye having an alkyl radical containing a carboxyl or sulfo group is apt to diffuse and spectrosensitize other silver halide layers. However, the combined use of sensitizing dyes to be used in this invention surprisingly provides a highly green sensitive emulsion layer with a strikingly reduced sensitization of the other layers.

On the other hand, it has been revealed in, for example, U.S. Pat. No. 2,913,329 that the combination of sensitizing dyes to be used in this invention provides a good result in the presence of a dispersion of color couplers. As shown in Example 3, however, it has been found that the combination of sensitizing dyes provides an unexpectedly great effect when the dye developers according to this invention are compared with the use of the coupler dispersion.

In the combined use of sensitizing dye and dye developer, the interaction of said sensitizing dye and said dye developer (the mechanism of said interaction is not explained theoretically and may be perhaps the desensitization effect due to the dye developer) results in a remarkably reduced sensitivity of a green emulsion. However the use of combination of specified sensitizing dyes to be used in this invention can lower said "interaction" to provide a highly green sensitive emulsion.

The use ratio of sensitizing dye represented by the general formula (I), (II) and (III), i.e., the ratio of sensitizing dye of the formula (I) to that of formula (II), the ratio of desensitizing dye of the formula (I) to that of formula (III) or the ratio of sensitizing dye of the formula (II) to that of formula (III) is not especially critical. However, it is especially effectively within the range of 9-1 : 1-9 by weight and may be varied according to the purpose of use.

The method for adding the sensitizing dye to the photographic emulsion is well known in the field for manufacturing a photographic emulsion. In general, it may be mixed as a solution in a solvent such as water, methanol, ethanol, methyl cellosolve and the like or added to the photographic emulsion. In this case, for the dissolution, a supersonic vibration may be used. The amount of sensitizing dye used may be varied according to the nature of each silver halide emulsion, the desired result, etc. In general for the optimum sensitization, 0.005 - 0.3 g of dye per g of silver halide is sufficient.

As silver halide emulsions to be used in this invention, there may be used silver halides such as silver chloride, bromide, iodobromide, chlorobromide and chloroiodobromide, and silver iodobromide.

While a conventional gelatin-silver halide emulsion is used in this invention, resinous materials which show no harm to the sensitive material or cellulose derivatives may be used instead of a part or all of the gelatin.

The photographic emulsion to be used in this invention may contain conventional additives such as chemical sensitizers, anti-foggants, stabilizers, film-

hardeners, coating assistants, plasticizers, development accelerators, air anti-foggants and the like, and may be coated in a common manner on a suitable supporter, e.g., glass, film of cellulose derivative, synthetic resin film, synthetic paper, Baryta paper, photographic paper coated with polyolefin film and the like.

The image-receiving element to be used in this invention consists of an image-receiving layer, which is alkali-permeable and can dye the dye developer from an alkaline solution, and a support. The image-receiving element comprises a support which is coated with at least one alkali-permeable and dyeable image-receiving layer. The image-receiving layer contains a reagent suitable for mordanting or has a function capable of fixing the diffused and unoxidized dye developer. The image-receiving material of said image-receiving layer and the constitution of said layer are well known in the art and are disclosed in Japanese Publication No. 29,756/61, 8,274/63 and 8,449/63, U.S. Pat. Nos. 3,003,872; 3,043,689; 3,065,074; 3,148,061; 3,239,337; 3,353,956; and 3,362,819.

In some cases, the dyeable layer comprises an alkali treating composition which is suitable to remain adhered to the support on stripping.

The support of said image-receiving element is preferably synthetic paper, papers such as Baryta paper, photographic paper coated with a polyolefin film, and glass, films of cellulose derivative and synthetic resin may be used.

This invention will be more fully illustrated by the following examples which are not intended to restrict the scope of this invention.

#### EXAMPLE 1

35 3g of magenta dye developer 4-isopropoxy-2-( $\beta$ -hydroquinonyl-ethyl)-phenylazo)-1-naphthol were dissolved in a mixed solvent of 6cc N,N-diethyl lauryl amide and 10cc ethyl acetate while heating at 70° C. The solution was dispersed in 50 cc of 10 percent gelatin containing 2cc of aqueous 5 percent sodium n-dodecylbenzenesulfonate to emulsify. The resulting emulsion was added with 2cc of 2 percent mucochloric acid and with water to make 100cc. The emulsion was coated on a support of cellulose triacetate so that the dried film thickness was 5 $\mu$ . A green sensitive iodobromide emulsion layer, which contained 4.8g of gelatin and  $3.5 \times 10^{-2}$  mols of silver per 100g of emulsion added with either single or the combination of the following sensitizing dyes, was coated thereon so that the dried film thickness was 2 $\mu$ . An emulsion, which was obtained by dissolving 1g of 4'-methyl phenyl hydroquinone in a mixed solvent of 2cc N,N-diethyl lauryl amide and 4cc ethyl acetate, emulsifying in 20cc of 10 percent aqueous gelatin solution containing 1cc of 5 percent aqueous sodium n-dodecylbenzenesulfonate solution, adding 2cc of 2 percent mucochloric acid and then adding water to make the whole 50cc, was coated thereon so that the dried film thickness might be 0.8 $\mu$ . The film was exposed to light behind an optical wedge having a continuously varied density, impregnated with the alkali reagent of the following compositions:

|                                          |        |
|------------------------------------------|--------|
| Hydroxyethyl cellulose of high viscosity | 3.5 g  |
| NaOH                                     | 4.0 g  |
| 1-Benzotriazole                          | 2.0 g  |
| 1-Phenethyl-2-picolinium bromide         | 2.0 g  |
| Water                                    | 100 cc |

allowed to stand for 2 minutes in contact with the following image-receiving sheet: a gelatin layer containing

a mixture of poly-4-vinyl pyridine mordant and 1-phenyl-5-mercaptopetetrazole coated on a Baryta support so that the dried film thickness was  $10\mu$  and then stripped to yield a positive color developer transfer positive color image, in which the density of area exposed to a large amount of light was low and that exposed to a small amount of light was high, on the image-receiving sheet. The reflection density of color image obtained on the image-receiving sheet was measured by means of a densitometer to determine the exposure amount at a reflection density of 1.0 and the results are shown in the Tables 1, 2-1, and 2-2. From the Tables, it can be seen that a high green sensitivity is obtained in this invention.

Table 1

| Test No. | Sensitizing Dye<br>(ml/100g emulsion) | Sensitivity <sup>11</sup> | Green Sensitivity<br>(only green <sup>22</sup><br>sensitive layer) |
|----------|---------------------------------------|---------------------------|--------------------------------------------------------------------|
| 1        | I - 1 (2)                             | 58.9                      | 95.5                                                               |
| 2        | do. (4)                               | 100                       | 100                                                                |
| 3        | do. (8)                               | 75.8                      | 100                                                                |
| 4        | III-1 (2)                             | 57.5                      | 103                                                                |
| 5        | do. (4)                               | 64.5                      | 112                                                                |
| 6        | do. (8)                               | 58.9                      | 112                                                                |
| 7        | I - 1(2) III-1(2)                     | 204                       | 151                                                                |
| 8        | do. (4) do. (2)                       | 229                       | 170                                                                |
| 9        | do. (4) do. (4)                       | 219                       | 148                                                                |

Tests No. 1 - 6 are controls.

The concentration of sensitizing dye solution is  $1 \times 10^{-3}$  mol/l.

<sup>11</sup> The sensitivity is the relative value of the inverse number of the exposure amount required for providing  $D = 1.0$ .

<sup>22</sup> Results after the black-and-white treatment of the sample, in which a green sensitive emulsion was coated on a cellulose triacetate. Fuji Filter No. 17 was used as the green filter.

Table 2

| Test No. | Sensitizing Dye<br>(ml/100 g emulsion) | Sensitivity <sup>11</sup> |     |
|----------|----------------------------------------|---------------------------|-----|
| 10       | I - 6 (2)                              | 70.7                      |     |
| 11       | do. (4)                                | 100                       |     |
| 12       | do. (8)                                | 95.5                      |     |
| 13       | III-2 (2)                              | 43.7                      |     |
| 14       | do. (4)                                | 49.6                      |     |
| 15       | do. (8)                                | 44.5                      |     |
| 16       | I - 6 (2)                              | III-2 (2)                 | 107 |
| 17       | do. (4)                                | do. (2)                   | 174 |
| 18       | do. (4)                                | do. (4)                   | 174 |
| 19       | II - 11 (2)                            | 63.1                      |     |
| 20       | do. (4)                                | 100                       |     |
| 21       | do. (8)                                | 70.7                      |     |
| 22       | III - 3 (2)                            | 50.1                      |     |
| 23       | do. (4)                                | 56.2                      |     |
| 24       | do. (8)                                | 52.5                      |     |
| 25       | II-11 (2)                              | III-3 (2)                 | 118 |
| 26       | do. (4)                                | do. (2)                   | 148 |
| 27       | do. (4)                                | do. (4)                   | 151 |
| 28       | I - 3 (2)                              | 87.0                      |     |
| 29       | do. (4)                                | 100                       |     |
| 30       | do. (8)                                | 100                       |     |
| 31       | II - 13 (2)                            | 89.0                      |     |
| 32       | do. (4)                                | 98.0                      |     |
| 33       | do. (8)                                | 98.0                      |     |
| 34       | I - 3 (2)                              | II - 13 (2)               | 123 |
| 35       | do. (4)                                | do. (2)                   | 126 |
| 36       | do. (4)                                | do. (4)                   | 120 |

<sup>11</sup> Same as in Table 1.

Test No. 10-15, 19-24 and 28-33 are controls.

### EXAMPLE 2

2g of yellow dye developer 1-phenyl-3-N-n-hexylcarboxyamido-4-(p-(2',5'-dihydroxyphenethyl)-phenylazo)-5-pyrazolone were dissolved in a mixed solvent of 2cc tricesyl phosphate and 5cc cyclohexanone with heating. The solution was emulsified in 50cc of 10 percent gelatin containing 2cc of 5 percent aqueous sodium n-dodecyl benzenesulfonate solution. The emulsion was added with 1cc of 2 percent aqueous 2-hydroxy-4,6-dichloro-S-triazine solution and then with

water to make the whole 100cc. The emulsion was coated on a cellulose triacetate support so that the dried film thickness was  $4\mu$ .

5 A green sensitive silver iodobromide emulsion layer, which contained 4.8g of gelatin and  $3.5 \times 10^{-2}$  mols of silver per 100g of emulsion added with either single or the combination of the following sensitizing dyes, was coated thereon so that the dried film thickness was  $2\mu$ .

10 An emulsion, which was obtained by dissolving 1 g of 4'-methylphenyl hydroquinone in a mixed solvent of 2cc N,N-diethyl-lauryl amide and 4cc ethyl acetate, emulsifying in 20cc of 10 percent aqueous gelatin solution containing 5 percent aqueous sodium

n-dodecylbenzenesulfonate solution, adding 2cc of 2 percent mucochloric acid and then adding water to make the whole 50cc, was coated on the layer so that the dried film thickness was  $0.8\mu$ .

35 The resulting film was treated in the same manner as in Example 1 to yield a transfer image of dye developer on an image-receiving sheet. The exposure amount at a reflection density of 1.0 is shown in the Table 3, from which it can be seen that a high sensitivity is obtained in this invention.

Table 3

| Test No. | Sensitizing Dye<br>(ml/100 g emulsion) | Sensitivity <sup>11</sup> |             |     |
|----------|----------------------------------------|---------------------------|-------------|-----|
| 37       | I - 6 (2)                              | 89.0                      |             |     |
| 38       | do. (4)                                | 100                       |             |     |
| 39       | do. (8)                                | 95.5                      |             |     |
| 50       | 40                                     | III - 1 (2)               | 52.5        |     |
|          | 41                                     | do. (4)                   | 56.2        |     |
|          | 42                                     | do. (8)                   | 51.2        |     |
|          | 43                                     | I - 6 (2)                 | III - 1 (2) | 141 |
|          | 44                                     | do. (4)                   | do. (2)     | 166 |
|          | 45                                     | do. (4)                   | do. (4)     | 170 |

55 <sup>11</sup> The sensitivity is indicated in the same manner as in the Table 1. The Tests No. 37 - 42 are controls.

### EXAMPLE 3

60 5g of cyan dye developer 5,8-dihydroxy-1,4-bis-[( $\beta$ -hydroquinonyl- $\alpha$ -methyl)ethylamino]anthraquinone were dissolved in a mixed solvent of 10cc N-n-butylacetanilide and 20cc methyl alcohol and the resulting solution was emulsified in 50cc of 10 percent gelatin containing 3cc of 5 percent sodium n-dodecylbenzenesulfonate.

65 The emulsion was added with 2cc of 2 percent aqueous 2-hydroxy-4,6-dichloro-S-triazine solution and then with water to make 100cc. The solution was coated on a cellulose triacetate support so that the

dried film thickness was  $5\mu$ . A silver iodobromide emulsion consisting of 20g of emulsion, which was obtained by dissolving 2.0g of 4'-methylphenyl hydroquinone in a mixed solvent of 2cc N-n-butylacetone and 4cc ethyl acetate and emulsifying in 20cc of 10 percent aqueous gelatin solution containing 1cc of 5 percent aqueous sodium n-dodecylbenzenesulfonate solution,  $4.7 \times 10^{-2}$  mols of silver per 100g of emulsion added with either single or the combination of the following sensitizing dyes and 5.3g of gelatin was coated thereon so that the dried film thickness was  $2.5\mu$ . 100cc of 3 percent gelatin containing 1cc of 2 percent 2-hydroxy-4,6-dichloro-S-triazine were coated thereon so that the dried film thickness was  $0.8\mu$ .

The film was treated in the same manner as in Example 1 to yield a transfer image of dye developer on an image-receiving sheet. The exposure amounts at a reflection density of 1.0 are shown in Table 4.

Table 4

| Test No. | Sensitizing Dye<br>(ml/100 g emulsion) | Sensitivity <sup>1)</sup> | Green Sensitivity<br>(only green sensitive<br>layer) <sup>2)</sup> |              |
|----------|----------------------------------------|---------------------------|--------------------------------------------------------------------|--------------|
|          |                                        |                           | Without Coupler                                                    | With Coupler |
| 46       | 1-4 (2)                                | 74                        | 97.5                                                               | 72.0         |
| 47       | do. (4)                                | 100                       | 100                                                                | 89.0         |
| 48       | do. (8)                                | 93.5                      | 89.0                                                               | 89.0         |
| 49       | III-1 (2)                              | 57.5                      | 74.0                                                               | 72.0         |
| 50       | do. (4)                                | 70.8                      | 91.0                                                               | 89.0         |
| 51       | do. (8)                                | 64.5                      | 91.0                                                               | 89.0         |
| 52       | 1-4 (2)                                | III-1 (2)                 | 252                                                                | 126          |
| 53       | do. (4)                                | do. (2)                   | 256                                                                | 135          |
| 54       | do. (4)                                | do. (4)                   | 256                                                                | 123          |

<sup>1)</sup> The sensitivity is indicated in the same manner as in Table 1. Tests No. 46 - 51 are controls.

<sup>2)</sup> Results after the black-and-white treatment of sample, in which a green sensitive emulsion was coated on cellulose triacetate. Fuji Filter No. 17 was used as green filter. In the Table, the same green sensitive emulsion as in the example was used in only the green sensitive layer without a coupler; for the layer with a coupler, an emulsion was used, in which 20 g/100 g emulsion of emulsified dispersion prepared by using 10 g of 1-hydroxy-N-n-dodecyl-2-naphthamide instead of a cyan dye developer in the preparation of a cyan dye developer emulsion were added to the same green sensitive emulsion.

## EXAMPLE 4

The following layers were coated in sequence on a cellulose triacetate support (10 in FIG. 2) to form a multi-layer film. FIG. 2 shows schematically the construction of the thus obtained film.

## (1) Cyan Developer Layer (9 in FIG. 2)

10g of 1,4-bis-( $\alpha$ -methyl- $\beta$ -hydroquinonyl-ethylamino)-anthra-quinone were dissolved completely in a mixed solvent of 10cc N,N-diethyl-lauryl amide and 20cc ethyl acetate with heating at  $60^\circ\text{C}$  for 20 min. The solution was emulsified in 100cc of 10 percent gelatin containing 10cc of 5 percent sodium n-dodecylbenzenesulfonate. The emulsion was added with 4cc of 2 percent 2-hydroxy-4,6-dichloro-S-triazine and then with water to make the whole 200cc and coated so that the dried film thickness was  $6.0\mu$ .

## (2) Red Sensitive Emulsion Layer (8 in FIG. 2)

A red sensitive silver iodobromide emulsion containing  $4.7 \times 10^{-2}$  mols/100g emulsion and 5.3g of gelatin was coated atop the cyan developer layer so that the dried film thickness was  $5.2\mu$ .

## (3) Intermediate Layer (7 in FIG. 2)

100cc of 5 percent gelatin containing 30g of emulsion, which was obtained by dissolving 3g of phenyl hydroquinone in a mixed solvent of 3cc N,N-diethyl lauryl amide and 8cc cyclohexane and emulsifying in 30cc of 10 percent gelatin containing 2cc of 5 percent sodium n-dodecylbenzenesulfonate, was coated atop the red sensitive emulsion layer so that the dried film thickness was  $4.2\mu$ .

## (4) Magenta Dye Developer Layer (6 in FIG. 2)

7g of 4-ethoxy-2-( $\beta$ -hydroxyethyl)-phenylazo)-1-

naphthol were dissolved in 7cc of N,N-diethyl lauryl amide and 14cc of ethyl acetate with heating and emulsified in 100cc of 10 percent gelatin containing 7cc of 5 percent sodium n-dodecylbenzenesulfonate. The emulsion was added with 4cc of 2 percent hydroxy-4,6-dichloro-S-triazine and then with water to make the whole 200cc and coated atop the intermediate layer (3) so that the dried film thickness was  $4.0\mu$ .

## (5) Green Sensitive Emulsion Layer (5 in FIG. 2)

A green sensitive emulsion, in which a silver iodobromide emulsion containing  $3.5 \times 10^{-2}$  mols per 100g of emulsion and 4.8g of gelatin added with a single or combination of the following sensitizing dyes, and was coated atop the magenta dye developer layer so that the dried film thickness was  $3.1\mu$ .

## (6) Intermediate Layer (4 in FIG. 2)

The same coating as shown in (3) above was coated

atop the green sensitive emulsion layer so that the dried film thickness was  $3.5\mu$ .

## (7) Yellow Dye Developer Layer (3 in FIG. 2)

5g of 1-phenyl-3-N-n-butylcarboxyamido-4-( $p$ -(2',5'-dihydroxy-phenethyl)-phenylazo)-5-pyrazolone were dissolved in a mixed solvent of 5cc N,N-diethyl lauryl amide and 14cc ethyl acetate and emulsified in 100cc of 10 percent gelatin containing 5cc of 5 percent sodium n-dodecylbenzenesulfonate. The emulsion was added with 4cc of 2 percent 2-hydroxy-4,6-dichloro-S-triazine and then with water to make the whole 200cc and coated atop the intermediate layer (6) so that the dried film thickness was  $3.4\mu$ .

## (8) Red Sensitive Emulsion Layer (2 in FIG. 2)

A blue sensitive silver iodobromide emulsion containing  $3.6 \times 10^{-2}$  mols per 100g of emulsion and 5.3g of gelatin was coated atop the yellow dye developer layer so that the dried film thickness was  $2.5\mu$ .

## (9) Protective Layer (1 in FIG. 2)

A liquid coating in which 100cc of the same coating as shown in (3) above were added with 4cc of 2 percent mucochloric acid, was coated atop the red sensitive emulsion layer so that the dried film thickness was  $1\mu$ .

A blue and red light were applied to the whole surface of the resulting film to expose the blue and red sensitive emulsion layer and the film placed behind an optical wedge having a continuously varied density was exposed to green light. The film was dipped in the alkali treating reagent described in Example 1, contacted to the image-receiving sheet described in Example 1 for 2 min. and then separated therefrom to yield a positive magenta dye developer transfer colored image on the

image-receiving sheet, said image having a dye density inversely proportional to the amount of light. The density of said image-receiving sheet was measured to determine the exposure amount for a density of 1.0 and the results are shown in Table 5, from which it can be seen that a high sensitivity may be obtained by the process of this invention.

Table 5

| Test No. | Sensitizing Dye<br>(ml/100 g emulsion) | Sensitivity <sup>a)</sup> |
|----------|----------------------------------------|---------------------------|
| 55       | I-1 (4)                                | 95                        |
| 56       | do. (8)                                | 100                       |
| 57       | III-1 (4)                              | 56                        |
| 58       | do. (8)                                | 63                        |
| 59       | I-1 (2)                                | 204                       |
| 60       | do. (4)                                | 269                       |
| 61       | do. (4)                                | 251                       |

<sup>a)</sup> The sensitivity is indicated in the same manner as in Table 1. Tests No. 55 - 58 are controls.

What is claimed is:

1. In a silver photographic emulsion for photographic sensitive material containing dye developers suitable for the diffusion transfer method, the improvement which comprises said photographic emulsion containing a green sensitizer comprising the combination of at least one of the sensitizing dyes represented by the formula (I):



wherein R is a member selected from the group consisting of a hydrogen atom and lower alkyl group, Y<sub>1</sub> and Y<sub>4</sub> each represent a member selected from the group consisting of a hydrogen atom, a lower alkyl group, a halogen atom, a hydroxyl group, an alkoxy group, an amino group, an acylamido group, an acyloxy group, a carbalkoxy group and an alkoxy carbonyl amino group, Y<sub>2</sub> and Y<sub>5</sub> each represent a member selected from the group consisting of a hydrogen atom, a lower alkyl group, a halogen atom, a hydroxyl group, an alkoxy group, an amino group, an acylamido group, an acyloxy group, a carbalkoxy group, an alkoxy carbonyl amino group and a phenyl group, Y<sub>3</sub> and Y<sub>6</sub> each represent a member selected from the group consisting of a hydrogen atom and an atomic grouping necessary for the formation of a benzene ring by the connection of Y<sub>3</sub> with Y<sub>2</sub> or of Y<sub>6</sub> with Y<sub>5</sub>, Y<sub>2</sub> and Y<sub>5</sub> each can be connected with Y<sub>1</sub> or Y<sub>4</sub>, respectively, to form a benzene ring with the proviso that both Y<sub>3</sub> with Y<sub>2</sub> and Y<sub>2</sub> and Y<sub>1</sub> do not form at the same time a benzene ring and both Y<sub>6</sub> with Y<sub>5</sub> and Y<sub>5</sub> with Y<sub>4</sub> do not form at the same time a benzene ring, R<sub>1</sub> and R<sub>2</sub> each represent a member selected from the group consisting of an alkyl group and a substituted alkyl group which is used in general for cyanine dyes, and at least one of said R<sub>1</sub> and said R<sub>2</sub> is an alkyl group containing a member selected from the group consisting of carboxy and sulfo group, X represents an anion and n is 1 or 2, such that n = 1 when said dye forms an intramolecular salt; and at least one of the sensitizing dyes represented by the following formula (II):



wherein R<sub>3</sub> is a member selected from the group consisting of a lower alkyl group and an allyl group, Y<sub>7</sub> is a member selected from the group consisting of a hydrogen atom and a halogen atom, Y<sub>8</sub> is a member selected from the group consisting of a hydrogen atom, a halogen atom, an alkoxy group, an amino group, an acylamido group, an acyloxy group and an alkoxy carbonyl amino group, Y<sub>9</sub> is a member selected from the group consisting of a hydrogen atom, a lower alkyl group, a halogen atom, a hydroxyl group and an alkoxy group, Y<sub>10</sub> is a member selected from the group consisting of a hydrogen atom, a lower alkyl group, a halogen atom, an alkoxy group, a phenyl group, a p-sulphophenyl group, a carboxyl group, an alkoxy carbonyl group, a cyano group and a trifluoromethyl group, Y<sub>11</sub> is a member selected from the group consisting of a hydrogen atom and an atomic grouping which is connected to Y<sub>10</sub> to form a benzene ring, Y<sub>9</sub> and Y<sub>10</sub> may be connected to form a benzene ring with the proviso that both Y<sub>9</sub> with Y<sub>10</sub> and Y<sub>10</sub> with Y<sub>11</sub> do not form at the same time a benzene ring, and R<sub>1</sub>, R<sub>2</sub>, X and n have the same meanings as in formula (I).

2. A silver halide photographic emulsion as claimed in claim 1 wherein the substituted alkyl group represented by R<sub>1</sub> or R<sub>2</sub> is selected from the group consisting of a hydroxy alkyl group, an acetoxyalkyl group, an alkoxyalkyl group, an alkyl group containing a carboxyl group, an alkyl group containing a sulfo group, an aralkyl group and an allyl group.

3. A silver halide photographic emulsion as claimed in claim 1 wherein the green sensitized combination is selected from combinations comprising sensitizing dyes of



and



4. A silver halide photographic emulsion as claimed in claim 1 wherein the dye developer contains a member selected from the group consisting of hydroquinonyl, o-dihydroxyphenyl and o- or p-amino-substituted hydroxyphenyl.

5. A silver halide photographic emulsion as claimed in claim 1 wherein the dye developer is selected from the group consisting of an azo dye developer and an anthraquinone dye developer.

6. A silver halide photographic emulsion as claimed in claim 5 wherein the dye developer is selected from

the group consisting of 4-isopropoxy-2-[p-( $\beta$ -hydroquinonylethyl)-phenylazo]-1-naphthol; 1-phenyl-3-N-n-hexylcarboxyamid-4-[p-(2',5'-dihydroxyphenethyl)phenylazo]-5-pyrazolone; and 5,8-dihydroxy-1,4-bis-[( $\beta$ -hydroquinonyl- $\alpha$ -methyl)-ethylamino]anthraquinone.

7. A silver halide photographic emulsion as claimed

in claim 1 wherein the silver halide is silver iodobromide.

8. A light-sensitive silver halide photographic material comprising an emulsion layer containing a silver halide photographic emulsion as claimed in claim 1.

\* \* \* \* \*

10

15

20

25

30

35

40

45

50

55

60

65